

Jan. 8, 1935.

L. J. MacGREGOR

1,986,937

QUOIT

Filed Sept. 10, 1932



FIG. 4.



FIG. 2.



FIG. 3.



LOUIS J MACGREGOR  
INVENTOR.

BY Eugene H Purdy  
his ATTORNEY



metal completely surrounds the circumference of the forging and defines two protuberant rings 4 and 5 disposed respectively upon its top and bottom sides. These rings are about one-eighth 5 of an inch in thickness, measured from the dotted line surface indicated in Fig. 4 which latter represents the normal finished surface of the quoit, and their width is such that they cover only 10 a comparatively small area upon the top and bottom of the forging.

The forging after initially being subjected to an annealing or normalizing operation to render the metal homogeneous throughout, as is well known in the art, is heated for about four hours 15 in an oxidizing atmosphere or flame at a temperature of about 1450 degrees F. so as to decarburize the outer surface of the forging and provide it with a skin or crust of soft metal. This crust need not penetrate beyond 1/32nd or 1/16th 20 of an inch and in any event ought not to exceed the thickness of the rings of metal 4 and 5. This decarburization treatment robs the surface of the forging of a large part of its carbon—in the case 25 of silico-manganese steel as specified the carbon content is reduced from approximately .50 per cent to approximately .20 per cent—but the interior metal of the forging is substantially unaffected by this treatment and retains its original relatively high carbon content.

Following decarburization, the forging is placed in a lathe and the protuberant rings of metal 4 and 5 are ground off by an abrasive wheel or other suitable means to a depth corresponding to the dotted line surface shown in Fig. 4 to expose 30 upon the circumference of the forging the interior metal constituting its core or body and which was not influenced by the preceding decarburization treatment. This circumferential rim of exposed metal while 35 harder than the surface covering on the top and bottom of the forging, is nevertheless too soft to satisfactorily constitute the edge of the quoit, so that further treatment is necessary to impart to it the requisite degree of hardness. The forging is therefore again heated, this time at a temperature of about 1600 degrees F. for about three-quarters of an hour, and then quenched in oil. By this operation the annulus of core metal which was brought to light by the removal of the rings 40 and 5 and which contains its original high percentage of carbon will take on an intense hardness; while the surface of the forging which was softened in the preceding decarburizing treatment and which is of relatively low carbon content—only about .20 per cent in the case of the 45 silico-manganese steel mentioned above—will be impervious to the treatment. Consequently the surface crust will remain substantially unchanged and will retain its former attributes.

After the second heating, the forging is again annealed and then ground to a surface finish of 1/16th of an inch upon the top and bottom of the quoit, the protuberant rings being removed by grinding with a coarse wheel. This surface finish is impervious to the action of acids and bases and is therefore relatively durable and less liable to 50 damage by impact or abrasion.

As the concluding step of this heat treatment, the forging is heated at a temperature of about 700 degrees F. for about two hours to impart to it the proper temper, in a manner which is well understood in the art, resulting in a quoit as 5 illustrated in Fig. 3, constituted of a core and circumferential edge of intense strength and hardness and a superficial crust of softer metal.

It is not necessary that the removal of the rings of excess metal precede the hardening and tempering step. For example, the method of the invention may be carried out by initially decarburizing the surface of the forging to impart to it a crust of soft metal, then hardening and tempering the body of the forging as before described. 10 The rings 4 and 5 will then be removed to develop the circumferential rim of hard metal. In this event however, the excess metal will be very 15 resistant because of prior hardening, but its removal may be accomplished by an abrasive wheel. 20 It is obvious that the crust or coating of soft metal may be applied to the forging in ways other than those which have been described. For example, this may be accomplished by dipping, by sherardizing or by electro-deposition, the circumference of the forging being cleared of the coating material in a subsequent operation. Or a 25 separate rim of hard metal may be shrunk onto the circumference of the forging. Such a novel form of quoit, irrespective of how produced, is 30 deemed to fall within the purview of this invention.

I claim:

1. A quoit having a core of relatively hard metal and a superficial crust of soft metal covering substantially the entire surface of the core, except upon its circumference.

2. A quoit having a core of relatively hard metal and a superficial crust of soft metal located a spaced distance inwardly of the circumference of the quoit.

3. A quoit having a core of relatively hard metal and a superficial crust of soft metal covering the major portion of its surface, the said core and crust being of the same kind of metal but of different degrees of hardness.

4. A quoit of disk form having a core of relatively hard metal and a thin superficial crust of soft metal integrally united with the core, said crust covering the upper and lower surfaces of the quoit and terminating a spaced distance from its circumference.

5. A steel quoit having a core of relatively high carbon content and a crust of relatively low carbon content covering the major portion of its surface.

LOUIS J. MACGREGOR,  
was most recently a member of the firm of *MacGregor, Clegg & Associates*, which firm was engaged in the preparation of this application. The inventor died on December 1, 1948, and was succeeded as counsel in connection with this application by the firm of *MacGregor, Clegg & Associates*, which firm is continuing to prosecute this application.

LOUIS J. MACGREGOR,  
was most recently a member of the firm of *MacGregor, Clegg & Associates*, which firm was engaged in the preparation of this application. The inventor died on December 1, 1948, and was succeeded as counsel in connection with this application by the firm of *MacGregor, Clegg & Associates*, which firm is continuing to prosecute this application.